

# UNITED STATES PATENT OFFICE.

SIMON STEVENS, OF NEW YORK, N. Y.

## IMPROVEMENT IN ROASTING AND DESULPHURIZING ORES AND MINERALS.

Specification forming part of Letters Patent No. 43,046, dated June 7, 1864.

*To all whom it may concern:*

Be it known that I, SIMON STEVENS, of the city and State of New York, have invented a new and useful Process of Roasting and Desulphurizing Ores and Minerals; and I do hereby declare that the following is a full and exact description of the same.

The nature of my invention consists, first, in using hydrocarbon vapors or gases as fuel for roasting and desulphurizing ores; secondly, in effecting the roasting and desulphurizing of ores by burning the vapors of hydrocarbons mixed or combined with either ordinary or superheated steam; and, thirdly, in the collecting from pyritous ores the gold and silver which they contain, by roasting or burning such ores in the flame from hydrocarbon vapors or gases, quenching the hot ore in water, then washing out and floating away the light earthy matters, and collecting the gold and silver by means of amalgamation with mercury, or on amalgamated plates, these several operations forming a continued process.

The ordinary mode of roasting ores is in heaps, mounds, ovens, or furnaces, using solid fuel, such as wood, coal, coke, or peat. For fuel I use volatile hydrocarbons, such as petroleum, coal-oil, earth-oil, or equivalent substances which may be easily converted into vapor by heat. By the combustion of such vapor mingled with air, or with air and steam, I effect the roasting and desulphurizing of ores and minerals, and in the case of the ores of the precious metals the roasting, washing, and amalgamating may be united, so as to form one continuous process.

I will now proceed to indicate the operations and apparatus necessary for carrying my invention into effect; but as these may be greatly varied, and do not form part of this invention, a brief description is deemed sufficient.

For converting the liquid hydrocarbon into vapor or gas any of the known devices for that purpose may be used. It is not necessary, or even preferable, to subject the liquid to destructive distillation so as to produce a permanent gas. The petroleum or liquid hydrocarbon is placed in a tank or reservoir, and by means of a tube conducted to a boiler or vessel to which heat may be applied, so as to convert the liquid into vapor or gas. This vapor may be mixed with air as it is produced; or the air may be

caused to mingle with it at the instant of combustion. Steam, common or superheated, may also be mixed with it in like manner, so as to regulate the combustion and assist in roasting and desulphurizing the ores. The combustion of vapors thus prepared is effected by devices already known, and therefore need not be particularly described.

The jets or burners used for delivering the vapor, air, and steam should be arranged in a row or series, so as to furnish the amount of heat required. The number of jets will depend upon the size of the furnace employed and the degree of heat necessary for effecting the roasting of the ore. By varying the relative proportions of hydrocarbon vapor, air, and steam, both the temperature and quality of the flame produced are always under the control of the workman.

The hydrocarbon vapor mixed with the proper amount of air for combustion being supplied in a series of jets, as already pointed out, the next thing is to bring the flame from such jets or the hot products of combustion in contact with the ore to be roasted. This may be done in many ways. The simplest is to place the pulverized ore on the hearth of an oven, or in a reverberatory furnace, so that the flame and heated gases may play upon it; or the ore may be broken into small pieces and placed in a revolving cylinder, such as is sometimes used for distilling coal, and the flame thrown through the cylinder as it revolves. The axis of the cylinder may be inclined, so as to cause the ore to pass through it as it is revolved. Other means may be used to move or stir the ore as it passes through the cylinder.

Another and in many respects a preferable mode of effecting the roasting of the ore is to bring it in fine powder into the flame. This may be accomplished by having the ore fed from a hopper, so as to fall into the flame from the row of gas or vapor burners, or by driving the ore into the flame with an air-blast; or the combustion may be carried on in an upright shaft or chimney, the gas or vapor jets being arranged in rows on one, two, or more sides of the shaft, either at the top or bottom of it; or when it is necessary to bring a large volume of flame in contact with the ore several parallel rows of jets may be arranged at different heights on the inside of the shaft. The ore in

fine powder is to be fed into the top of the shaft or chimney, and as it falls it will be completely roasted by the flame or hot gases and vapors. Steam or superheated steam may be injected through the jets which convey the hydrocarbon vapors. Air also, for supporting combustion, may be mingled with oil vapor; or it may be introduced through separate pipes.

When ores of the precious metals, as pyrites containing gold, are roasted by my process, the entire operation of roasting, washing, and amalgamating the gold may be carried on in a continuous manner. As the ore is roasted, it should fall into water, where, by stirring and agitating, it is washed, and the light and earthy matters carried off by a current of water. The heavier parts containing gold and silver will settle to the bottom, and may be combined with mercury or collected on amalgamated plates in any of the usual modes well known to miners and metallurgists. As the hot ore falls directly into the water, the latter will be kept at a high temperature, and therefore the amalgamation of the precious metals will be readily effected.

Having thus described my invention and the several modes in which it may be applied, what I claim, and desire to secure by Letters Patent of the United States, is—

1. The use of hydrocarbon vapors or gases as fuel in the roasting and desulphurizing of ores or minerals.

2. The desulphurizing and roasting of ores by means of a combined blast or current of hydrocarbon vapor, air, and steam, applied in the manner substantially as herein set forth.

3. The process herein described of separating and collecting the precious metals from pyritic ores, which process consists in roasting and desulphurizing the ore, receiving it while hot in water, washing and removing the light earthy matters, and amalgamating the precious metals, these several operations forming a continuous process, as above set forth.

SIMON STEVENS.

Witnesses:

MUNROE CHUBB,  
GEO. P. WILLEY.